

J. C. RUSSELL.

METAL ARTICLE.

APPLICATION FILED DEC. 30, 1912.

1,080,590.

Patented Dec. 9, 1913.



Witnesses:

J. W. Mayfield

J. B. Humphries.

Inventor:

James C. Russell  
By J. M. Cooke  
attorney.

# UNITED STATES PATENT OFFICE.

JAMES C. RUSSELL, OF PITTSBURGH, PENNSYLVANIA.

## METAL ARTICLE.

1,080,590.

Specification of Letters Patent. Patented Dec. 9, 1913.

Application filed December 30, 1912. Serial No. 739,191.

*To all whom it may concern:*

Be it known that I, JAMES C. RUSSELL, a resident of Pittsburgh, in the county of Allegheny and State of Pennsylvania, have invented a new and useful Improvement in Metal Articles; and I do hereby declare the following to be a full, clear, and exact description thereof.

My invention relates to railroad rails and other steel articles and has special reference to such a quality of article wherein the crystalline structure of the metal comprising the same will be broken up and the rail thus rendered tough and durable and unlikely to become broken by any sudden shocks or changes in atmospheric conditions.

The object of my invention is to provide a cheap, simple and efficient form of railroad rail which will be treated in such a manner that the same will be adapted to be used on any kind of a road and will, on account of its tough durable nature, tend to eliminate the frequent and numerous accidents of the present day caused by the breaking of such railroad rails.

My invention consists, generally stated, in the novel quality of railroad rail and other steel articles, wherein the interior of the same is composed of hard material known as martensite while the outer surface or exterior of the same consists of a soft, tough material known as troostite, although no break line between the different qualities will be apparent, as they gradually blend into one another.

My improved railroad rail and other similar articles such as bars, rods, etc., are subjected to treatment in an apparatus similar to that described in my U. S. Letters Patent, No. 993,411, granted May 30th, 1911, for an improvement in apparatus for treating railroad rails and other like articles.

It is well known that in the present method of rolling and manufacturing steel railroad rails the finished articles are likely to become broken by any sudden shock or by any sudden change in the atmospheric conditions so that by the breaking of rails on railroad tracks trains are derailed, passengers oftentimes killed or injured by reason thereof on account of the heretofore imperfect, inherent, nature of the same. It

is also well known that in the present quality of railroad rail used throughout the country the molecules composing the same generally appear to form a simple, homogeneous substance, but when placed under a microscope are seen to be a conglomeration of crystals of different substances. This crystallization, or, what is known as crystalline structure, is broken up in my improved article and the whole really made to be what it appears to the naked eye in the old rail, viz., a solid, simple homogeneous mass of metal.

My invention covers the treating of steel having .30 or greater per cent. carbon, and is intended to produce a metal which will be soft and tough on the exterior and hard on the interior, in order that the same cannot be cracked or particles chipped from the same and the tough exterior of the same will hold the inner particles together and prevent the whole article from becoming disrupted or broken.

Steel when heated to a temperature of about seven or eight hundred degrees centigrade will present a bright cherry red appearance and will be in what is known as austenite condition. If this steel were allowed to cool slowly to atmospheric temperature it would revert to its original quality, which is known as pearlite, although a few molecules of the austenite would remain. The presence of carbon in the steel will tend to prevent the reversion of the entire mass from austenite to pearlite, so that high carbon steel in slowly cooling will sometimes retain as much as 70% austenite molecules. If, for instance, the steel could contain no carbon whatsoever it would revert from austenite to pearlite absolutely. During the change from austenite to pearlite steel will pass through several transition stages which are not, under ordinary circumstances, permanent conditions or qualities of steel. When steel has been heated to austenite and is then allowed to cool it will first change to martensite. If it then continues to cool it will change from martensite to troostite and from troostite it will change to pearlite, although, as before mentioned, the presence of carbon in the steel will prevent some of the molecules from reverting to pearlite.

To enable others skilled in the art to

which my invention appertains to treat and use my improved railroad rail and other steel articles I will describe the same more fully referring to the accompanying drawing in which the figure shows a steel railroad rail during the process of treatment.

The process by which I obtain my improved steel article is as follows:—The rail or other article which has been treated to 10 austenite is first passed into a bath of oil and passes slowly through such bath so that entirely passing through the same consumes but a few seconds of time. The rail then continues in a bath of oil but water is forced 15 at a pressure through the oil and against the surface of the head of the rail so that by the time the rail emerges from the baths in the trough it is cooled almost to atmospheric temperature. When the rail or bar A is 20 first passed into the oil bath its condition is austenite and as it continues through this bath the outer part *a* of the same, to a depth of about one-sixteenth of an inch, is brought down to troostite condition, while the ma- 25 terial *b* within the inner layer is not as yet affected by the liquid bath. Now if the rail were at this point taken from the bath the hot inner metal of the same would bring the outer surface back to a red heat and the 30 whole would be austenite at a temperature of about one hundred degrees, or thereabout, less than when entering the bath. But instead of withdrawing the rail it is allowed to continue through the oil bath *c* but water 35 *d* is forced under pressure against the head of the same from pipes *g*. The rail during this stage of the treatment is shown in the drawing. As it is subjected to this bath or treatment the outside layer *a* of the same 40 being in a troostite condition, while the inner metal *b* is still in an austenite condition, the action of cold water *d* upon the surface of the same will tend to "trap" or hold the troostite material in this same condition, while the rapid cooling of the inner 45 austenite will bring the same to martensite. This is effected by the action of the cold water on the head of the rail and the martensite is "trapped" in the interior just as the troostite is "trapped" on the exterior. The web and flange of the rail A are 50 allowed to pass through the oil bath, unaffected by water until they are almost entirely troostite, whereupon the water is 55 forced against said web and flange to trap the troostite so that there is only a small portion of martensite present. Thus the finished material will be martensite on the interior and troostite on the exterior. This 60 will give a material having a hard body covered by an outside layer or exterior of tough durable steel, and homogeneous throughout as to its chemical characteristics.

65 Materials having a soft interior and a hard

exterior have been made but they are objectionable in many ways because the hard outer surface can be cracked or particles chipped from the same, while in my improved rail or other article the outer material of troostite will form a tough durable inclosure for the hard metal so that it cannot be chipped or broken and the troostite will tend to hold the particles or molecules comprising the martensite interior firmly 70 together.

75 It is possible to carry out this treatment and produce my improved article without using an oil bath. This is accomplished by using first, a bath of warm or hot water and 80 this will bring the outer surface down to a troostite condition—then a bath of warm water having cold water under pressure forced through the same and against the surface of the article. This will tend to 85 "trap" the troostite and will also "trap" the martensite within the same.

90 Although it is possible to obtain my improved article by using water baths of different temperatures, I prefer the oil treatment as the water after being forced through the oil and against the surface of the article will immediately seek its level and pass downward through the oil where it will be carried off as explained in my United 95 States patent referred to above.

100 It will be readily seen that on account of the oil maintaining the higher level and the cold water being forced in at all times the oil will become heated to a higher temperature as it will retain a great deal of the heat from the rail or article passing through it. The liquids being at different 105 temperatures will tend to prevent the material from changing from austenite to pearlite and by breaking up the crystalline structure will produce a material superior to any heretofore manufactured and one which numerous tests and experiments have shown to withstand shocks which would break the 110 ordinary similar article before such treatment. In fact in the case of a rail placed under test before and after treatment, such as described, my new article was formed to withstand a shock twice as great as that 115 necessary to fracture the article before treatment. The need of an article of this kind, particularly in railroad construction, has long been felt as such a rail will tend materially to eliminate the great number of 120 wrecks which have been caused by the breaking of railroad rails, and the consequent derailing of trains, and will also decrease the weight of railroad rails as lighter rails may be used. It will at once be seen that the 125 article produced by this treatment will be of such a quality that the outside of the same will be soft and tough troostite while the inside or center of such article will be of a hard martensite material, which will 130

allow the same to bend double without fracturing it. It will also be seen that steel of any shape or size may be thus treated and the article produced will have the qualities 5 hereinbefore mentioned.

What I claim as my invention and desire to secure by Letters Patent is:—

• A steel article homogeneous as to its chemical characteristics having its exterior com-

posed of tough material and its interior of 10 hard material.

In testimony whereof, I the said JAMES C. RUSSELL have hereunto set my hand.

JAMES C. RUSSELL.

Witnesses:

T. B. HUMPHRIES,  
J. N. COOKE.